

1

2,878,192

**REFORMING CATALYST**

Armand J. de Rosset, Clarendon Hills, and Vladimir Haensel, Hinsdale, Ill., assignors to Universal Oil Products Company, Des Plaines, Ill., a corporation of Delaware

No Drawing. Application July 17, 1953  
Serial No. 368,826

8 Claims. (Cl. 252—442)

This invention relates to a reforming process and to the manufacture of catalysts for use therein.

The term "reforming" is well known in the petroleum industry and refers to the treatment of gasoline fractions to improve the antiknock characteristics thereof. The petroleum fraction that is upgraded in reforming may be a full boiling range straight run gasoline having an initial boiling point within the range of from about 50° F. to about 100° F. and an end boiling point within the range of from about 350° F. to about 425° F. It may also be a natural gasoline as obtained from the refining of natural gases or it may be any selected fraction of the natural gasoline. The natural gasoline or the natural gasoline fraction will have an initial boiling point and an end boiling point substantially the same as that of the gasoline hereinbefore described. In the reforming process the gasoline fraction that is selected usually is the higher boiling fraction, commonly referred to as naphtha, and generally will have an initial boiling point of from about 150° F. to about 250° F. and an end boiling point within the range of from about 350° F. to about 425° F. The catalyst of the present invention may also be applied to the reforming of cracked gasoline or mixtures of cracked and straight run and/or natural gasoline. Reference to gasoline in the present specification, therefore, means a full boiling range gasoline or any fraction thereof, and also that the gasoline fraction may contain components boiling above the gasoline range.

In the reforming process there are four major reactions. The first is an aromatization reaction in which naphthalene hydrocarbons are converted to aromatics. The second is a dehydrocyclization reaction in which the straight chain or slightly branched chain paraffins are cyclized to form aromatics. Third is an isomerization reaction in which straight chain or slightly branched chain paraffins are converted to more branched chain paraffins. This reaction occurs as a result of a strain put upon a carbon to carbon bond so that there is a shift of a carbon atom in the molecule to form a more branched chain molecule. In this specific reaction there is no change of molecular weight. The reaction may also be characterized as increasing the number of methyl groups in the hydrocarbon molecule. The fourth is a cracking reaction in which the heavier straight chain or slightly branched chain paraffins, which have low antiknock characteristics, are converted to lighter straight chain or branched chain paraffins which have higher antiknock characteristics. When this last reaction is conducted in the presence of hydrogen, the unsaturated hydrocarbon that is formed as a result of the cracking operation, is saturated to the paraffin by reaction with hydrogen in the presence of the reforming catalyst. The cracking or splitting of the carbon to carbon bond is one of the more important reactions in a successful reforming process. It is necessary that the splitting of the carbon to carbon bond be controlled so that there is no excessive formation of normally gaseous products. For example, it would be possible to crack a C<sub>10</sub> hydrocarbon to form

2

ten molecules of methane, however, unless methane is the specifically desired product, it would be uneconomical in a reforming process to crack the C<sub>10</sub> hydrocarbon to form methane. It is more desirable to crack a C<sub>10</sub> hydrocarbon so that two molecules of pentane are formed and it would be still more desirable if, during the reaction, isomerization would simultaneously take place so that the product obtained would be isopentane. It is an object of the present invention to provide a catalyst wherein the cracking activity is controlled and selective so that excessive amounts of normally gaseous products are not produced in a reforming process.

Uncontrolled or non-selective cracking results in the more rapid formation of larger quantities of coke or carbonaceous matter which deposits on the catalyst and decreases or destroys its activity to catalyze the desired reactions. This in turn results in shorter processing cycles or periods with the necessity of more frequent regeneration of the catalyst by burning the carbonaceous products therefrom, or should the catalyst activity be destroyed it will be necessary to shut down the unit to remove the old catalyst and replace it with new catalyst.

Another important feature in a successful reforming process is the matter of hydrogen production and consumption. Investigation has shown that the presence of hydrogen in the reforming zone further tends to decrease the amount of carbonaceous deposit on the catalyst. In view of the fact that the cost of hydrogen is quite high, it is essential that there be no net consumption of hydrogen or, in other words, at least as much hydrogen must be produced in the process as is consumed therein.

While the catalyst of the present invention is particularly suitable for the reforming of gasoline, it is understood that this novel catalyst may be utilized for the conversion of other hydrocarbon fractions. Thus the catalyst may be used for the dehydrogenation of selected hydrocarbon fractions such as naphthalene to produce aromatics including, specifically, the dehydrogenation of cyclohexane to benzene, methylcyclohexane to toluene, ethylcyclohexane to ethylbenzene, etc., the dehydrogenation of paraffins to produce the corresponding olefins, including, specifically, dehydrogenation of butane to butene, pentane to pentene, hexane to hexene, etc., the dehydrogenation mono-olefins to produce the corresponding di-olefins including, specifically, dehydrogenation of butene to butadiene, pentene to pentadiene, etc. The catalyst may also be utilized to effect dehydrocyclization reactions including, specifically, the conversion of normal hexane to benzene, normal heptane to toluene, etc. The catalyst may also be used for effecting isomerization reactions including the isomerization of normal or mildly branched chain paraffins, the isomerization of alkyl cyclic compounds to isomers thereof, including the isomerization of methylcyclopentane to cyclohexane, ethylcyclopentane to methylcyclohexane, etc., the isomerization of alkyl benzenes, etc. Furthermore, the catalyst may be used for effecting hydrogenation reactions including non-destructive hydrogenation, as for example, the hydrogenation of butene to butane, pentene to pentane, aromatics to cycloparaffins, etc., and destructive hydrogenation of heavier oil to gases and/or gasoline fractions. In still another embodiment the catalyst of the present invention may be used for effecting oxidation of hydrocarbons to form the corresponding oxides, such as the oxidation of normal butene to normal butyl alcohol. The catalysts are also very effective for desulfurizing sulfur-containing fractions. The desulfurization may be effected in the presence or absence of hydrogen. In the desulfurization reaction the organic sulfur compounds such as mercaptans or thiophenes are converted to hydrogen sulfide which may be stripped out in subsequent operations.

In one embodiment the present invention relates to a method of preparing a catalyst which comprises commingling alumina with a solution of a platinum compound containing a water soluble acidic compound not substantially reactive with the alumina at impregnating conditions, and with a solution of hydrogen fluoride containing a water soluble acidic compound not substantially reactive with the alumina at impregnating conditions, said platinum compound being in an amount to form a final catalyst containing from about 0.01% to about 1% by weight of platinum, and said hydrogen fluoride being in an amount to form a final catalyst containing from about 0.1% to about 8% by weight of combined fluorine.

In another embodiment the present invention relates to a method of preparing a catalyst which comprises commingling with alumina a solution of a platinum compound, hydrogen fluoride and a water soluble acidic compound not substantially reactive with the alumina at impregnating conditions, said platinum compound being in an amount to form a final catalyst containing from about 0.01% to about 1% by weight of platinum, and said hydrogen fluoride being in an amount to form a final catalyst containing from about 0.1% to about 8% by weight of combined fluorine.

In a specific embodiment the present invention relates to a method of preparing a catalyst which comprises commingling with dry precipitated alumina particles of definite size and shape, a solution containing chloroplatinic acid, hydrogen fluoride and a sufficient amount of a water soluble acidic compound not substantially reactive with the alumina at impregnating conditions to lower the pH, said chloroplatinic acid being in an amount to form a final catalyst containing from about 0.01% to about 1% by weight of platinum, and said hydrogen fluoride being in an amount to form a final catalyst containing from about 0.1% to about 8% by weight of combined fluorine, and calcining the thus treated alumina particles.

In a further embodiment the present invention relates to a process for reforming a gasoline fraction which comprises subjecting said fraction to contact at reforming conditions with a catalyst prepared by commingling with alumina a solution of a platinum compound, hydrogen fluoride and a water soluble acidic compound not substantially reactive with the alumina at impregnating conditions to lower the pH, said platinum compound being in an amount to form a final catalyst containing from about 0.01% to about 1% by weight of platinum, and said hydrogen fluoride being in an amount to form a final catalyst containing from about 0.1% to about 8% by weight of combined fluorine, and calcining.

Platinum-containing catalysts and various methods of manufacture have heretofore been suggested. These catalysts have been of limited commercial acceptance because of the high cost thereof. It has been found that exceptionally good platinum-containing catalysts are prepared in accordance with the novel features of the present invention. While these catalysts may contain larger concentrations of platinum which may range up to about 10% by weight or more of the alumina, it has been found that exceptionally good catalysts may be prepared to contain from as low as about 0.01% to about 1% by weight of platinum. Catalysts of these low platinum concentrations are particularly preferred in the present invention because of the considerably lower cost of the catalyst and thus enhances the attractiveness of the catalyst for use in commercial processes.

However, in order to obtain improved results with these low platinum concentrations, it is necessary that a particular type of supporting component be composited with the platinum, especially when the support contains halogen in specific amounts. It has been found that alumina shows unexpected advantages for use as a supporting component for the low platinum concentration and low halogen concentration, apparently due to some peculiar

association of the alumina with the platinum and with the halogen either as a chemical combination or as a physical association. Platinum-halogen on other supports such as alumina-silica, alumina-titania, alumina-magnesia and alumina-boron oxide also shows catalytic activity and the method of our invention for compositing platinum and halogen with the alumina may also be used for compositing platinum and halogen with these other alumina-containing components, but not necessarily with equivalent results. When the halogen is combined with the combination such as alumina-silica, the halogen reacts with both the alumina and the silica, however, the silica-halogen compound may vaporize from the catalyst and thus the catalyst will not contain a silica-halogen compound such as, specifically, silicon, tetrafluoride, but will contain the aluminum halide.

As another essential feature of the present invention impregnation of the alumina must be effected in the presence of an acidic compound which may be an inorganic acid, an organic acid and/or an acid acting salt. A particularly suitable method of impregnation is by means of a solution of a suitable platinum compound. However, it has been found that unless the impregnation is effected in the presence of an acidic compound uneven distribution 20 of the platinum and the fluorine in or on the alumina particles is obtained. Usually this uneven distribution comprises surface coating, that is, the platinum compound and fluorine are distributed on only the surface of the particles and not evenly throughout the mass. By 25 effecting the impregnation in the presence of an acidic solution, even distribution of the platinum and fluorine throughout the alumina particles is obtained. Catalysts containing a non-uniform distribution of the platinum and fluorine are not satisfactory apparently due to a 30 peculiar association of the platinum and halogen and alumina which is required to produce satisfactory catalysts. It appears that a particular spacial arrangement of the platinum in relation to the alumina and to each other is necessary in order to obtain satisfactory catalysts. 35 The desired arrangement is not achieved when the platinum atoms are grouped too closely to the others or are spaced at too great a distance apart. In any event, the use of an acid along with chloroplatinic acid and hydrogen fluoride results in a solution which is used for compositing with the alumina in accordance with this invention.

Heretofore it has been suggested that a basic compound be added to the platinum-containing solution prior to compositing with the support. Specifically, ammonium hydroxide was added to a solution of chloroplatinic acid and the theory set forth was that the ammonia associated itself with the chloroplatinic acid forming a complex which in turn homogeneously distributed itself throughout the alumina. We have now discovered that 50 when the commingling of the platinum compound and hydrogen fluoride with the alumina is performed in an acidic solution, a uniformly impregnated composite results. One explanation, although we do not intend our invention to be limited thereto, is that the presence of the acid tends to keep the chloroplatinic acid solution in a non-ionized form and therefore the platinum compound instead of associating itself with the surface of the alumina particles thoroughly impregnates the alumina particles to produce a final catalyst in which the platinum is uniformly distributed throughout the alumina. This 55 explanation is also applicable to the beneficial effect noted when impregnating the alumina with the fluoride. Hydrogen fluoride is a weak acid in comparison to acids such as hydrochloric and nitric and, therefore, when an acid such as nitric acid is added to a solution of hydrofluoric acid, the ionization of hydrofluoric acid to the hydrogen ion and the fluoride ion is suppressed. Therefore, by the 60 presence of an acid, the hydrogen fluoride is rendered more inactive, that is, it is present more as the molecule HF and the hydrogen fluoride will more thoroughly im-

pregnate the alumina particles before reacting with the alumina.

The acidic compound that is selected must be one that is not substantially reactive with the alumina at impregnating conditions, and preferably is one that is not substantially reactive with the alumina at any of the conditions in which it is in contact with the alumina during the preparation of the catalyst. In some cases only certain concentrations of the acidic compound are substantially reactive with the alumina and these concentrations should not be used. An acidic compound may be used, however, when it is reactive with the alumina, if the resultant product or residue is not harmful to the catalyst and/or if the resultant product or residue is removed in a further treatment, such as washing or calcination, and/or if the formation of the resultant product or residue does not harm the final catalyst. It is preferred, however, that the acidic compound be water soluble and substantially unreactive with the alumina. In most cases it may be removed by washing or by calcination. Most concentrations of aqueous solutions of hydrogen halides and specifically hydrogen fluoride and/or hydrogen chloride are reactive with the alumina and therefore they are not to be used as the acidic compound of our invention. Likewise higher concentrations of sulfuric acid, especially at elevated temperature are reactive with the alumina and these higher concentrations and elevated temperatures are not to be used when employing sulfuric acid. Usually the impregnation is done at a concentration and temperature such that the sulfuric acid is not reactive with the alumina and at these concentrations and temperatures it may be used.

A particularly satisfactory method of impregnating the alumina with the platinum comprises the use of an aqueous solution of chloroplatinic acid containing a water soluble acidic compound not substantially reactive with the alumina at impregnating conditions. In one embodiment the acidic compound is added to chloroplatinic acid and the mixture is added to the alumina particles. Subsequently an acidic compound not substantially reactive with the alumina at impregnating conditions, is added to an aqueous solution of hydrogen fluoride and the mixture is added to the alumina particles. The reverse procedure may also be used, that is, the alumina may first be impregnated with the fluoride-acidic compound containing solution and subsequently impregnated with the platinum-acidic compound containing solution. In still another embodiment the alumina may be calcined before impregnating with any one or with both of the solutions and also the alumina after commingling with the halogen-containing solution may be calcined before commingling with the platinum-containing solution, and likewise the alumina after commingling with the platinum-containing solution may be calcined before contacting with the halogen-containing solution. In any event, the mixture is allowed to stand, preferably with or after suitable agitation so that thorough mixing is obtained and even distribution of the platinum and halogen throughout the alumina particles is effected. The invention therefore, is directed to the use of an acidic compound not substantially reactive with the alumina at commingling conditions. When commingling alumina with a platinum-containing compound and hydrogen fluoride, the alumina may be commingled with a solution containing both the platinum-containing compound and hydrogen fluoride in the presence of the acidic compound, or else the alumina may be impregnated with the platinum-containing solution first, followed by impregnating with the fluoride-containing solution, or, as hereinabove set forth, the reverse procedure may be used.

The solution of platinum-compound and acidic compound may be prepared in any suitable manner. Chloroplatinic acid is the preferred platinum compound to be used in accordance with the present invention because of its ready availability and lower cost. It is understood

that other platinum compounds may be used in accordance with the present invention, however, not necessarily with equivalent results. As hereinbefore set forth, the amount of platinum compound utilized is preferably controlled so that the final catalyst contains from about 0.01% to about 1% by weight of platinum.

A solution of platinum compound, hydrogen fluoride and acidic compound may also be prepared in any suitable manner. The order of mixing of these compounds is usually not important in that there does not appear to be any substantial chemical reaction involved when mixing these compounds, other than the usual ionization, that is, no new gaseous compound is evolved during the mixing, or no precipitate forms during the mixing.

Any suitable acidic compound may be used within the scope of the present invention. When preparing the solution of the platinum compound and acidic compound, the preferred acidic compounds comprise the acids, nitric acid, sulfuric acid, phosphoric acid and aluminum nitrate. Other suitable acids include acetic acid, oxalic acid, formic acid, propionic acid and more generally include acids and acid salts which are more acidic than chloroplatinic acid or any other platinum-containing compound that is selected. Mixtures of acidic compounds may also be used within the scope of this invention. As hereinbefore set forth the acidic compound must not be substantially reactive with the alumina at concentrations or at temperatures as herein set forth. When preparing the solution of platinum compound, hydrogen fluoride and acidic compound or the solution of hydrogen fluoride, and acidic compound, the preferred acidic compounds usually comprise the stronger acids since it is believed that one of the beneficial effects of an acidic compound is to suppress the ionization of hydrogen fluoride to render it more inactive with the alumina and, therefore, the acidic compound must be chosen with the view to suppressing the ionization of hydrogen fluoride. The preferred acidic compounds therefore to use when hydrogen fluoride is present comprise the acids, nitric acid, sulfuric acid, and phosphoric acid. While the organic acids which include acetic acid, oxalic acid, formic acid, and propionic acid may be used, they are not as suitable since they do not as actively suppress the ionization of hydrogen fluoride as the aforementioned acids. Mixtures of acidic compounds may also be used in the hydrogen fluoride containing impregnating solution.

The amount of acidic compound required will vary with the particular acidic compound and with the particular solution utilized. In general only a small amount of acidic compound will be required and usually will be in amount sufficient to lower the pH of the platinum-containing solution to below 2.5 and preferably below 2.0. When the impregnating solution contains hydrogen fluoride the amount of acidic compound will more usually be in amount sufficient to lower the pH of the solution to below about 1.0.

The amount of acidic compound that is to be added may be measured by the amount necessary to lower the impregnating solution to a specified pH. The preferred method is by measuring a stoichiometric amount of acidic compound that is added to the platinum-containing solution and/or to the halogen-containing solution and/or to the platinum and halogen-containing solution. The pH of the solution containing the hydrogen fluoride does not change much upon the addition of a small amount of acidic compound since the hydrogen fluoride acts as a weak acid and the ions of hydrogen and fluorine combine to form the hydrogen fluoride molecule. The same effect is noticed when adding small amounts of acid to chloroplatinic acid solutions. The concentration of acidic compound will be within the range of from about 0.001 to about 5.0 molar with respect to said acidic compound and preferably from about 0.005 to about 3.0 molar. Concentrations below this wider range are too weak to be

effective and concentrations above this range often are too reactive with the alumina.

The alumina for use in the present invention may be prepared in any suitable manner. A particularly preferred method is to prepare alumina by adding a suitable reagent, such as ammonium hydroxide, ammonium carbonate, etc., to a salt of aluminum such as aluminum chloride, aluminum nitrate, aluminum acetate, etc., in an amount to form aluminum hydroxide which, upon drying is converted to alumina and in the interest of simplicity, the aluminum hydroxide is referred to as alumina in the present specification and claims in order that the percentages are based on the alumina free of combined water. It has been found aluminum chloride is generally preferred as the aluminum salt, not only for convenience in subsequent washing and filtering procedures, but also because it appears to give best results.

After the alumina has been formed it is generally washed to remove soluble impurities. Usual washing procedures comprise washing with water, either in combination with filtration or as separate steps. It has been found that filtration of the alumina is improved when the wash-water includes a small amount of ammonium hydroxide. The severity of washing will depend upon the particular method employed in preparing the catalyst. In one embodiment of the invention the alumina is thoroughly washed with a suitable amount of water and preferably water containing ammonium hydroxide to reduce the chlorine content of the alumina to below about 0.1%. In another embodiment of the invention this washing may be selective to retain chloride ions in an amount of from about 0.2% to about 8% by weight of the alumina on a dry basis. In general, it is preferred to wash the alumina thoroughly and if it is desired to add chlorine it is added as a separate step because better control of the amount of chlorine is obtained in this manner.

In some cases it is desirable to prepare the catalyst in the form of pills of uniform size and shape and this may readily be accomplished by grinding the partially dried alumina cake with a suitable lubricant such as stearic acid, rosin, graphite, etc. and then forming the pills in any suitable pelleting or extrusion apparatus. The halogen may be added before or after forming the alumina into particles of uniform size and shape. In still another embodiment the halogen and platinum addition may be effected prior to forming the composite into particles of uniform size and shape.

Alumina spheres may be continuously prepared by passing droplets of an alumina sol into an oil bath maintained at an elevated temperature and retaining the droplets in said oil bath until the droplets set to gel spheres. The spheres are continuously withdrawn from the oil bath and immediately thereafter aged prior to being contacted with water or aqueous solutions. The spheres may then be dried and calcined at a temperature of from about 500° F. to 1400° F. or more.

As hereinbefore set forth the platinum and the halogen may be composited with the alumina in three ways. In one method the alumina is impregnated with a solution of a platinum compound containing the acidic compound. In the second method the alumina is impregnated with a solution of hydrogen fluoride containing an acidic compound. In the third method the alumina is impregnated with a solution of platinum compound, hydrogen fluoride and the acidic compound.

The solution of platinum and acidic compound may be composited with the alumina in any suitable manner. When the solution is to be composited with the alumina in a wet condition, this is readily accomplished by adding the solution to the alumina and thoroughly mixing the same to obtain uniform distribution after which the composite is washed and the washed material is dried at a temperature of from about 200° F. to about 500° F. for a period of from about 2 to 24 hours or more. It is also

possible to add the acidic compound to the alumina prior to the addition of the solution of the platinum compound, however, the platinum-containing compound and the acidic compound are more usually mixed before compositing with the alumina. When particles of irregular size and shape are desired, the dried material may be ground and then calcined at a temperature of from about 700° F. to about 1100° F. for a period of from about 2 to 12 hours or more. On the other hand, when particles of uniform size and shape are desired a suitable lubricant, such as stearic acid, rosin, hydrogenated coconut oil, graphite, etc. are added to the dried material and then it is formed into particles of uniform size and shape by any suitable method such as pelleting, extrusion, etc. The particles are then calcined at a temperature within the range as hereinbefore set forth. The manner of compositing the solution of platinum compound and acidic compound with the alumina, as hereinabove set forth, is also used when the alumina is previously composited with the fluorine.

The solution of hydrogen fluoride and acidic compound may be composited with the alumina in any suitable manner. The hydrogen fluoride is a form which will readily react with the alumina and the presence of the acidic compound not substantially reactive with the alumina at commingling conditions, produces an alumina-fluoride composite in which the fluorine is more uniformly distributed than when the acidic compound is absent. An aqueous solution of hydrogen fluoride can be easily handled and by its use the specific amount of fluoride to be added may be easily controlled.

The concentration of hydrogen fluoride in the finished catalyst will be within the range of from about 0.1% to about 8%. The fluoride ion however, appears to be very active when reforming certain gasoline fractions and the higher concentrations are not as desirable and therefore the preferred range of fluoride concentration is from about 0.1% to about 3% by weight of the alumina on a dry basis. Concentrations of fluorine above 3% sometimes adversely effect the selectivity of the catalyst, thus catalyzing side reactions to an extent greater than desired.

The solution of platinum compound, hydrogen fluoride and acidic compound may be composited with the alumina in substantially the same manner as hereinabove set forth. The amount of hydrogen fluoride present will be controlled so that the amount of fluoride present on the final catalyst will fall within the range of from about 0.1% to about 8% by weight of the final catalyst, and likewise the amount of platinum compound will be controlled so that the amount of platinum on the final catalyst will be within the range of from about 0.01% to about 1% by weight. When this solution is used the amount of acidic compound present is that amount wherein the concentration of the acidic compound in the impregnating solution lies within the range of from about 0.001 to about 5.0 molar with respect to said acidic compound.

In a preferred embodiment of the invention the alumina prior to commingling with the other components is formed into particles of definite size and shape. This is accomplished in substantially the same manner as hereinbefore set forth, but before the platinum is composited with the alumina, the alumina particles may be calcined at a somewhat higher temperature which may range from about 500° F. to about 1400° F. Commingling of any of the hereinbefore mentioned solutions may be accomplished in any suitable manner including soaking the alumina pills in the solution and either draining off the excess solution or heating to remove the volatilizable materials. Another suitable method is by dipping the alumina particles in the solution. In any event the alumina is contacted with the solution for a sufficient period of time to obtain uniform distribution of the solution throughout the alumina after which the composite may be dried at a temperature of from about 200° F. to

about 500° F. for a period from about 2 to 24 hours or more and then calcined at a temperature of from about 700° F. to about 1100° F. for a period of from about 2 to 12 hours or more. The upper temperature limit of 1100° F. is necessary when the alumina is already composed with the platinum, however, when the composite is alumina-halogen or alumina itself, the calcination may be performed in a temperature range of from about 500° F. to about 1400° F. for a period of from about 2 to 24 hours or more. In another embodiment the alumina is combined with a halogen and the alumina-halogen composite may be treated as hereinabove set forth. The calcination is preferably effected in the presence of air or other oxygen-containing gas. In another embodiment of the invention the calcination may comprise a two-stage method in which it is first calcined in the presence of hydrogen followed by calcination in air or the reverse procedure may be used.

In some cases the lubricant may be removed during the high temperature heating. In other cases, as for example, when graphite is used as the lubricant the separate high temperature heating step may be omitted and the effective heat treatment of the catalyst may be obtained in the plant before or during processing of the hydrocarbon.

Although the catalyst of the present invention will have a long life, it may be necessary to regenerate the catalyst after long periods of service. The regeneration may be effected by treatment with air or other oxygen-containing gas to burn carbonaceous deposits therefrom. Generally it is preferred to control the regeneration temperature not to exceed 1000° F. and preferably the regeneration is effected at a temperature within the range of from about 600° F. to about 900° F.

The exact operating conditions used when employing the catalyst of this invention will depend upon the character of the charging stock as well as the activity of the catalyst being used, however, the conditions usually will be in the following ranges: Temperatures from about 500° F. to about 1000° F., a pressure of from about 50 to about 1000 p. s. i. or more, a weight hourly space velocity (defined as the weight of oil per hour per weight of catalyst in the reaction zone) of from about 0.5 to about 20 or more. The reforming is preferably effected in the presence of hydrogen which may be introduced from an extraneous source or recycled within the process. In one embodiment of the process sufficient hydrogen will be produced in the reforming reaction to furnish the hydrogen required in the process and, therefore, it may be unnecessary to either introduce hydrogen from an extraneous source or to recycle hydrogen within the process. However, it usually will be preferred to introduce hydrogen from an extraneous source at the beginning of the operation and to recycle hydrogen within the process in order to be assured of a sufficient hydrogen atmosphere in the reaction zone. The hydrogen present in the reaction zone will be within the range of from about 0.5 to about 20 mols of hydrogen per mol of hydrocarbon. In some cases the gas to be recycled will contain hydrogen sulfide introduced with the charge or liberated during the reaction and it is within the scope of the present invention to treat the hydrogen-containing gas to remove hydrogen sulfide or other impurities before recycling the hydrogen within the process.

Other selected processing conditions are required depending upon the particular reaction desired. For example, for dehydrogenation of normal butane the temperature should be within the range of from about 800° F. to about 1100° F., the pressure from about atmospheric to about 50 lbs. per sq. inch, and the gaseous hourly space velocity from about 200 to about 5000. For hydrogenation reactions the temperature may range from atmospheric to about 500° F., the pressure from about 100 to about 3000 lbs. per sq. inch or more and the weight hourly space velocity from about 0.5 to 5.

Processes using the catalyst of the present invention may be effected in any suitable equipment. The finished catalyst may be deposited as a fixed bed in a reactor and the hydrocarbons to be treated are passed therethrough in either upward or downward flow. The catalyst may be used in a fluidized type of operation in which the catalyst and hydrocarbons are maintained in a state of turbulence under hindered settling conditions, or a fluidized fixed bed type of operation may be used in which the catalyst and hydrocarbons are maintained in a state of turbulence under hindered settling conditions but where catalyst is not withdrawn from or introduced into the reaction zone during the processing cycle. The catalyst may also be used in the moving bed type of process in which the catalyst and hydrocarbons are passed either in concurrent or countercurrent flow through a reaction zone, and the catalyst may also be used in the suspensoid type of operation in which the catalyst and hydrocarbons are passed as a slurry through the reaction zone. The reactants from any of the hereinbefore mentioned reaction zones are normally subjected to a further treatment, such as the stabilization of the product to separate normally gaseous paraffins therefrom to obtain a final reformed product of the desired volatility and vapor pressure.

The following examples are given to further illustrate the novelty and utility of the present invention, but are not given for the purpose of unduly limiting the generally broad scope of the present invention.

#### EXAMPLE I

A catalyst was prepared by adding ammonium hydroxide to aluminum chloride hexahydrate to form aluminum hydrate. The resultant aluminum hydrate was washed thoroughly in order to reduce the chloride content to below 0.1% by weight on a dry basis. The alumina was dried at a temperature of about 340° F. for 8-10 hours and the partially dried alumina was ground, Stearotex added as a lubricant, and then pilled in a Stokes pelleting machine to form cylindrical pills of  $\frac{1}{8}$ " x  $\frac{1}{8}$ " in size. The pills were then calcined in air at a temperature of about 1232° F. for 3 hours. The pills were then submerged in an aqueous solution containing chloroplatinic acid, hydrogen fluoride, and nitric acid. The nitric acid was used in an amount so that the impregnating solution was 1.5 molar in nitric acid. The solution was used in concentration and amount to produce a final catalyst containing 0.49% platinum and 0.31% fluorine. This catalyst is referred to as catalyst A.

Another catalyst, referred to as catalyst B, was prepared in substantially the same manner as catalyst A, however, nitric acid was omitted from the impregnating solution. After impregnation the mixtures were evaporated to dryness and the pills subsequently calcined in air at a temperature of about 932° F. for approximately 3 hours.

Catalysts A and B were used for reforming a Mid-Continent naphtha having an initial boiling point of 210° F. and an end boiling point of 390° F. The conditions maintained in the reforming zone were an average catalyst temperature of 860° F., a pressure of 500 lbs. per sq. inch, a liquid hourly space velocity of about 2 and a hydrogen to hydrocarbon mol ratio of about 3.1. An analysis of the reformed products are shown in the following table.

Table I

|                              | Catalysts | A     | B     |
|------------------------------|-----------|-------|-------|
| 70 Octane No. F-1 Clear..... |           | 87.9  | 85.5  |
| Dispersion @ 20° C.....      |           | 112.5 | 111.9 |

The dispersion value is a measure of the aromatic content of the gasoline and it may easily be seen that catalyst A, as prepared according to the method of our

invention, had superior aromatizing properties. The octane number of the product produced by catalyst A is also substantially higher than that produced using catalyst B.

## EXAMPLE II

Alumina pills are prepared as outlined in Example I. The pills are then submerged in an aqueous solution containing chloroplatinic acid, hydrogen fluoride, and sulfuric acid. The sulfuric acid is used in an amount so that the solution is 0.50 molar with respect to the sulfuric acid. The solution is in a concentration and amount to produce a final catalyst containing 0.3% platinum and 0.4% fluorine. This catalyst is referred to as catalyst C. Catalyst D is prepared in a similar manner except sulfuric acid is not used. The platinum and halogen of catalyst C will be more evenly distributed than the platinum and halogen of catalyst D. Catalyst C will also maintain its activity for a longer period of time than catalyst D when they are used in a reforming process.

## EXAMPLE III

A catalyst is prepared by calcining alumina pills at 1232° F. for approximately 3 hours. The alumina pills are submerged in a solution of 4.8% hydrofluoric acid to which nitric acid is added in an amount to make the solution 0.5 molar with respect to the nitric acid. The solution is prepared and used in an amount so that the final catalyst will contain 0.5% by weight of fluoride based on the alumina on a dry basis. The pills and solution are evaporated to dryness and are then submerged in a solution of chloroplatinic acid containing nitric acid in an amount to lower the pH of the solution to about 1.5. The solution and pills are again evaporated to dryness and calcined in air at a temperature of 932° F. for 3 hours.

An inspection of the final catalyst shows that the halogen and the platinum are distributed very evenly through the pills. This catalyst is referred to as catalyst E.

Another catalyst is prepared in substantially the same manner except that the nitric acid is left out of the chloroplatinic acid solution. This catalyst is referred to as catalyst F.

Catalysts E and F are treated with a stream of hydrogen sulfide to convert the platinum into platinum sulfide which is a dark color. An inspection of catalysts E and F shows that the platinum in catalyst E is much more evenly distributed through the catalyst mass. The platinum of catalyst F is found on the surface of the alumina pills with little penetration into the center of the pill.

The catalysts may be used for reforming a Mid-Continent naphtha having an initial boiling point of 190° F. and an end boiling point of 390° F. Over an extended period of operation the activity of catalyst E will remain higher than the activity of catalyst F.

We claim as our invention:

1. In the manufacture of a catalyst comprising plati-

num, alumina and fluorine, the improvement which comprises impregnating alumina with a solution containing chloroplatinic acid, hydrogen fluoride and an additional mineral acid selected from the group consisting of nitric, 5 sulfuric and phosphoric acids, the concentration of said mineral acid and the impregnating temperature being such that there is no substantial reaction between the alumina and mineral acid during the impregnation, the hydrogen fluoride being in an amount to form a final catalyst containing from about 0.1% to about 8% by weight of combined fluorine and said additional acid being in an amount to lower the pH of said solution to below 2.5.

2. The improvement as defined in claim 1 further characterized in that the amount of said mineral acid is 15 sufficient to lower the pH of the solution to below about 1.0.

3. The improvement as defined in claim 1 further characterized in that said solution is from about 0.001 to about 5.0 molar with respect to said mineral acid.

20 4. The improvement as defined in claim 1 further characterized in that said mineral acid is nitric acid.

5. The improvement as defined in claim 1 further characterized in that said mineral acid is sulfuric acid.

6. The improvement as defined in claim 1 further characterized in that said mineral acid is phosphoric acid.

7. In the manufacture of a catalyst comprising platinum, alumina and fluorine, the improvement which comprises impregnating alumina with a solution containing a platinum compound and hydrogen fluoride in sufficient 30 amounts to form a final catalyst containing from about 0.01% to about 1% by weight of platinum and from about 0.1% to about 8% by weight of combined fluorine, said solution additionally containing at least one acid selected from the group consisting of nitric, sulfuric and phosphoric acids in an amount to impart to the solution a pH value below about 1.0.

8. In the manufacture of a catalyst comprising platinum, alumina and fluorine, the improvement which comprises impregnating alumina with a solution containing a 40 platinum compound and hydrogen fluoride in sufficient amounts to form a final catalyst containing from about 0.01% to about 1% by weight of platinum and from about 0.1% to about 8% by weight of combined fluorine, said solution additionally containing at least one acid selected from the group consisting of nitric, sulfuric, phosphoric, acetic, oxalic, formic and propionic acids in an amount to impart to the solution a pH value below about 1.0.

## References Cited in the file of this patent

## UNITED STATES PATENTS

|              |                 |       |                |
|--------------|-----------------|-------|----------------|
| 2,331,915    | Kirkpatrick     | ----- | Oct. 19, 1943  |
| 2,479,109    | Haensel         | ----- | Aug. 16, 1949  |
| 2,611,736    | Haensel         | ----- | Sept. 23, 1952 |
| 55 2,636,863 | Haensel         | ----- | Apr. 28, 1953  |
| 2,753,310    | Riedl           | ----- | July 3, 1956   |
| 2,769,688    | Milliken et al. | ----- | Nov. 6, 1956   |